

## UNITED STATES PATENT OFFICE

2,286,112

## WAX DECOMPOSITION INHIBITOR

Albert A. Schilling, Stratford, Conn., and George H. Latham, Wilmington, Del., assignors to Remington Arms Company, Inc., a corporation of Delaware

No Drawing. Application June 26, 1940,  
Serial No. 342,442

11 Claims. (Cl. 117—158)

This invention relates to means to prevent the decomposition of hot wax. More particularly, it relates to an inhibitor to be used in a hot wax bath, said bath being kept at an elevated temperature for process purposes. As an example of the use of the present invention, paper shot shell tubes may be impregnated with a paraffin wax in such a bath. The wax bath into which the paper tubes are dipped for impregnation is kept at a temperature of between 230 and 240° F. (110°—115.5° C.), so that the wax is liquid and will readily penetrate the paper. The elevated temperature is necessary to secure the proper penetration of the wax in the paper. When a wax, such as a paraffin wax, is kept at this temperature in a tank for an extended period, acidic decomposition products are formed and, although it is not precisely known, it is believed that these are in the form of organic acids and probably anhydrides and lactones. The presence of the decomposition products prevents the proper penetration of the wax into the paper tubes and thereby decreases the resistance of the paper tube to the burning powder. If the powder burns through the tube, failure of the tube will result, and, upon extraction of the fired shell from the gun, a part of the tube will be left in the barrel. The degree of the decomposition can be measured by determining the saponification value of the wax. This decomposition also results in loss of a large amount of wax and causes a loss of time in the reclaiming and correction of the condition of the decomposed wax. This loss of wax may be attributed to the volatilization of the volatile decomposition products, to the discarding of the entire lot of the wax being used or to the discarding of the sweatings after purifying the decomposed wax. Another difficulty that is prevented by the use of the inhibitor of this invention is the lowering of the melting point of the wax by the decomposition. When no inhibitor is used, oily decomposition products accumulate in the wax which lower the melting point. This is of particular importance in shot shell tubes because the lower melting point will allow the wax to migrate into the powder of the shot shell, at a lower temperature, thereby materially affecting and decreasing the efficiency of the powder. It is possible that this is a matter of surface tension. Previously, it was necessary to replace part of the old wax with a fresh wax at sufficiently frequent intervals to prevent the saponification value from going above, for example, 10 or 12, whereas with the inhibitor of the present invention it is possible to use the

same wax for a considerable length of time. It has been found desirable in general to keep the saponification value below 10 or 12, although it is to be understood that it is not limited thereto. 5 The saponification value may be determined by any standard method such as that disclosed on page 388 of "Chemical Technology and Analysis of Oils, Fats and Waxes" by Lewkowitsch (6th ed., vol. I). Many materials have been tried for the purpose of preventing the decomposition of the wax, but most of these were found to be unstable at the temperature used, thereby giving a dark brown or black color, or resulting in a sludge formation. Some substances used also 10 showed a tendency to cause tarnishing of the brass shot shell head and to develop a foul odor in the wax. It has been found that by the use of poly-alkylated phenol and especially poly-methyl phenol, that the decomposition of the wax bath is inhibited. In the catalytic synthesis of methanol from carbon monoxide and hydrogen, a mixture of poly-alkylated phenols is produced. These are producible by the high pressure catalytic hydrogenation of carbon monoxide and include, among other things, 2-6 dimethyl and 2-4-6 trimethyl phenol. It is also possible to redistill this mixture of poly-alkylated phenols and use the redistilled product as the inhibitor. 15 20 25

It has been found that as low as .2% of the inhibitor may be added to the wax bath to give good results.

The following table is a summary of results obtained with the inhibitor of this invention in a crude scale paraffin wax, in comparison with 30 the untreated wax:

| Amount of mixture of poly-alkylated phenols; percent of wax | Saponification value |           |           |
|-------------------------------------------------------------|----------------------|-----------|-----------|
|                                                             | 72 hours             | 141 hours | 230 hours |
| 40                                                          |                      |           |           |
| 0.50                                                        | 0                    | 0         | 0.5       |
| 1.00                                                        | 0.7                  | 0.8       | 0.4       |
| 0                                                           | 10.0                 | 14.0      | 29.0      |

45 It is to be understood that the example given of the impregnation of paper shot shell bodies in the wax bath is merely for purposes of illustration and that the hot wax bath may be employed for other uses, such as, for example, other wax impregnated paper articles or any other place where a wax bath must be maintained at elevated temperatures. By this invention a 50 method of preventing a bothersome and expensive decomposition of a hot wax bath has been devised. As many different embodiments of this

invention may be made without departing from the scope thereof, it is to be understood that the invention is not limited to the embodiment given except as defined by the appended claims.

What is claimed is:

1. The method of inhibiting the decomposition of a hot wax bath comprising adding thereto a poly-methyl phenol.

2. The method of inhibiting the decomposition of a hot wax bath comprising adding thereto a mixture including poly-methyl phenols.

3. The method of inhibiting the decomposition of a hot wax bath comprising adding thereto a 2-4-6 trimethyl phenol.

4. The method of inhibiting the decomposition of a hot wax bath comprising adding thereto a mixture including 2-6 dimethyl phenol and 2-4-6 trimethyl phenol.

5. The method of inhibiting the decomposition of a hot wax bath comprising adding thereto at least .2% of poly-methylated phenols.

6. The method of inhibiting the decomposition of a hot wax bath comprising adding thereto at least .2% of a mixture including 2-6 dimethyl phenol and 2-4-6 trimethyl phenol.

7. The method of inhibiting the decomposition of a molten paraffin wax bath maintained at an elevated temperature of about 230° to 240° F. (110°-115.5° C.), which comprises incorporating therein at least 0.2% of the mixture of 2:6-dimethyl phenol and 2:4:6-trimethyl phenol.

8. The process of impregnating with paraffin wax the paper tubes of shot shells, while preventing the formation therein of materials which may cause migration of the impregnating material from the paper tubes to the powder in loaded shot shells, and which may also tarnish the brass heads of said shells which comprises immersing the paper tube in a hot paraffin wax bath to

which has been added at least 0.2% of its weight of polymethylated phenol material maintained at a temperature of 230°-240° F. (110°-115.5° C.) until the paper is impregnated with the bath material.

9. The process of impregnating with paraffin wax the paper tubes of shot shells, while preventing the formation therein of materials which may cause migration of the impregnating material from the paper tubes to the powder in loaded shot shells, and which may also tarnish the brass heads of said shells which comprises immersing the paper tube in a hot paraffin wax bath in which has been incorporated at least 0.2% of its weight of a 2:4:6-trimethyl phenol-2:6-dimethyl phenol mixture maintained at a temperature of 230°-240° F. (110°-115.5° C.) until the paper is impregnated with the bath material.

10. The process of impregnating with paraffin wax the paper tubes of shot shells, while preventing the formation therein of materials which may cause migration of the impregnating material from the paper tubes to the powder in loaded shot shells, and which may also tarnish the brass heads of said shells which comprises immersing the paper tube in a hot paraffin wax bath in which has been incorporated at least 0.2% of its weight of 2:4:6-trimethyl phenol maintained at a temperature of 230°-240° F. (110°-115.5° C.) until the paper is impregnated with the bath material.

11. The method of impregnating paper shot shells with wax, which comprises dipping the paper shot shells into a wax bath comprising essentially molten paraffin wax and at least 0.2% of polymethylated phenol.

ALBERT A. SCHILLING.  
GEORGE H. LATHAM.